

1,011,659.

E. H. STRANGE.  
MANUFACTURE OF VARNISHES.  
APPLICATION FILED FEB. 26, 1910.

Patented Dec. 12, 1911.



WITNESSES  
M. E. Blair  
a. C. Powell

INVENTOR  
EDWARD HALFORD STRANGE

By Horson and Horson  
Attorneys

# UNITED STATES PATENT OFFICE.

EDWARD HALFORD STRANGE, OF STAPLE INN, LONDON, ENGLAND, ASSIGNOR OF ONE-HALF TO EDMUND RISOLIERE BURRELL, OF MILLWALL, LONDON, ENGLAND.

## MANUFACTURE OF VARNISHES.

1,011,659.

Specification of Letters Patent. Patented Dec. 12, 1911.

Application filed February 26, 1910. Serial No. 546,050.

*To all whom it may concern:*

Be it known that I, EDWARD HALFORD STRANGE, M. Sc., a subject of the King of Great Britain and Ireland, of 7 Staple Inn, 5 in the county of London, England, have invented new and useful Improvements in the Manufacture of Varnishes, of which the following is a specification.

This invention relates to the process of 10 making varnish, in which process hard gum, or resin, commonly known as copal, is heated with a solvent under pressure in a digester, without any linseed, or like, oil being present during digestion. Such a process is described in U. S. Letters Patent to Strange and Graham 708,935, Sept. 9, 1902. In the said process more solvent is employed in the digester for dissolving the copal than is necessary to be present in the 15 finished varnish, and owing to the great pressure generated in this digester at the temperature required for effecting solution (usually a pressure of between 450 and 600 lbs. to the square inch), a digester of a very 20 cumbrous and expensive character has to be provided to give the requisite strength to withstand the pressure, especially as, at the high temperature employed, steel is liable to have its normal strength lessened, and the 25 process is therefore, to a corresponding extent, dangerous and expensive.

Objects of this invention are to make the process quite safe and also cheaper and the plant very much less cumbrous and expensive.

An apparatus is diagrammatically illustrated in the accompanying drawing in which the process may be carried out.

According to the present invention, instead of using a completely closed digester A, I employ a digester which is provided with a distilling head, or pipe, or the equivalent B, which is kept open so as to give, during the whole of the dissolving process, 40 communication between the digester and an outlet, preferably to a condenser C, the outlet valve D being regulated so that the pressure in the digester does not exceed two hundred and fifty lbs. to the square inch, 45 or thereabout, this pressure being a convenient and safe one to work at. In working under these conditions, with, say, four parts by weight of copal and one part by 50 weight of solvent, a complete solution of the

copal can be obtained before the whole of 55 the solvent has been volatilized.

In the specifications of the aforesaid prior patents, it is stated that an excess of volatile solvent is employed, but, according to the process of the present invention, much less 60 solvent is required than will be required in the varnish manufactured; for instance, the solution can be effected with as little as about one-tenth of the weight of solvent required in the finished varnish. This enables 65 solvents to be employed, for effecting the solution of the copal, which it is desirable shall not be present, or not present to any objectionable extent, in finished varnish of good quality; for instance, volatile fractions 70 of the distillation of shale oil, or of petroleum, known as "turpentine substitute", can be employed for effecting the solution of the copal in the digester, these being very efficient and much cheaper than American 75 turpentine, and they do not decompose, or give rise to objectionable products by prolonged heating and, by the time the solution is completed under the aforesaid conditions, the proportions of such solvent to 80 dissolved copal is very small. The solvent necessary for making the finished varnish of the requisite consistency is preferably American turpentine, which, being added at a lower temperature, will not have its odor, 85 or other valuable property, injuriously affected by the heat of the dissolving process, but, if desired, for commoner varnishes, volatile solvents, such as fractions of the distillation of petroleum, or of shale oil, can 90 be used instead of turpentine to make the finished varnish of the requisite consistency.

A further advantage of this invention is that when American turpentine is used in the digester as the solvent in accordance 95 with the process of the aforesaid specifications, objectionable products are liable to be formed and the odor of the American turpentine is affected, and although it may not affect the practical utility of the varnish, 100 the absence of this odor of American turpentine is prejudicial to the sale of the finished varnish and, as in the process according to this invention, the turpentine is added subsequently to dissolving and at a lower temperature, no objectionable products are formed therefrom and the desirable odor 105 of the turpentine is retained.

If the varnish is to be an oil varnish, instead of a spirit varnish, linseed oil is added after the treatment in the digester and at a temperature of, say, about 100° centigrade. If it be required to filter, or allow impurities to settle, this can be effected after the product from the digester has been thinned sufficiently for this purpose and, in the case of oil varnishes, before the oil is added.

Driers may be added to the varnishes if desired.

What I claim is:—

1. The process of manufacturing varnish which comprises the step of dissolving copal by heating the latter under pressure but not materially in excess of 250 pounds to the square inch, in the presence of a quantity of a volatile solvent less than required in the finished product.

2. The process of manufacturing varnish which comprises the step of dissolving copal by heating the latter under pressure but not materially in excess of 250 pounds to the square inch, in the presence of a quantity of a volatile solvent less than required in the finished product and simultaneously distilling off the solvent.

3. The process of manufacturing varnish, which comprises the step of dissolving copal by heating the latter under pressure but not materially in excess of 250 pounds to the square inch, in the presence of a relatively small quantity of mineral oil distillation.

4. The process of manufacturing varnish, which comprises the step of dissolving copal by heating the latter under pressure but not materially in excess of 250 pounds to the square inch, in the presence of a relatively small quantity of mineral oil distillation and simultaneously distilling off the solvent.

5. The process of manufacturing varnish,

which comprises the step of dissolving copal by heating the latter under pressure but not materially in excess of 250 pounds to the square inch, in the presence of a quantity of a volatile solvent less than required in the finished product and simultaneously distilling off the solvent and thereafter adding the requisite quantity of solvent.

6. The process of manufacturing varnish, which comprises the step of dissolving copal by heating the latter under pressure but not materially in excess of 250 pounds to the square inch, in the presence of a quantity of a volatile solvent less than required in the finished product and simultaneously distilling off the solvent and thereafter at a lower temperature adding the requisite quantity of solvent.

7. The process of manufacturing varnish, which comprises the step of dissolving copal by heating the latter under pressure but not materially in excess of 250 pounds to the square inch, in the presence of a quantity of a volatile solvent less than required in the finished product and simultaneously distilling off the solvent and thereafter thinning and filtering.

8. The process of manufacturing varnish, which consists in dissolving copal by heating the latter under pressure but not materially in excess of 250 pounds to the square inch, in the presence of a relatively small quantity of mineral oil distillation, simultaneously distilling off the solvent and thereafter at a lower temperature adding the requisite quantity of turpentine for the finished product.

In testimony whereof I have signed my name to this specification, in the presence of two subscribing witnesses.

EDWARD HALFORD STRANGE.

Witnesses:

JOHN ROWLAND WHINCOP,  
H. D. JAMESON.